



US008137577B2

(12) **United States Patent**  
**Kaneko et al.**

(10) **Patent No.:** **US 8,137,577 B2**  
(45) **Date of Patent:** **Mar. 20, 2012**

(54) **REFRIGERATOR OIL COMPOSITION, AND  
REFRIGERATOR COMPRESSOR AND  
REFRIGERATION SYSTEM USING THE  
COMPOSITION**

(75) Inventors: **Masato Kaneko**, Chiba (JP); **Hiroaki  
Koshima**, Chiba (JP)

(73) Assignee: **Idemitsu Kosan Co., Ltd.**, Tokyo (JP)

(\*) Notice: Subject to any disclaimer, the term of this patent is extended or adjusted under 35 U.S.C. 154(b) by 102 days.

(21) Appl. No.: **12/097,884**

(22) PCT Filed: **Dec. 14, 2006**

(86) PCT No.: **PCT/JP2006/324955**

§ 371 (c)(1),  
(2), (4) Date: **Jun. 18, 2008**

(87) PCT Pub. No.: **WO2007/072733**

PCT Pub. Date: **Jun. 28, 2007**

(65) **Prior Publication Data**

US 2009/0277212 A1 Nov. 12, 2009

(30) **Foreign Application Priority Data**

Dec. 20, 2005 (JP) ..... 2005-367051

(51) **Int. Cl.**

*C09K 5/04* (2006.01)  
*F25B 43/02* (2006.01)

(52) **U.S. Cl.** ..... **252/68; 62/468**

(58) **Field of Classification Search** ..... **252/68;  
62/468**

See application file for complete search history.

(56) **References Cited**

U.S. PATENT DOCUMENTS

5,185,092 A \* 2/1993 Fukuda et al. ..... 508/440  
5,512,198 A \* 4/1996 Sasaki et al. ..... 252/68  
5,514,292 A \* 5/1996 Sato et al. ..... 252/68

5,547,593 A \* 8/1996 Sanechika et al. ..... 508/207  
5,686,398 A \* 11/1997 Minokami et al. ..... 508/481  
5,858,930 A \* 1/1999 Desai et al. ..... 508/261  
5,918,269 A \* 6/1999 Mahaffey, Jr. ..... 73/40.7  
6,123,009 A \* 9/2000 Kanayama et al. ..... 92/71  
6,245,725 B1 \* 6/2001 Tanaka et al. ..... 508/365  
6,906,191 B2 \* 6/2005 Koshima et al. ..... 544/374  
8,043,523 B2 \* 10/2011 Kaneko ..... 252/68  
2001/0012821 A1 \* 8/2001 Koishikawa et al. ..... 508/416  
2003/0018198 A1 \* 1/2003 Koshima et al. ..... 548/110  
2004/0180796 A1 \* 9/2004 Iwata et al. ..... 508/103  
2009/0159836 A1 \* 6/2009 Kaneko ..... 252/68

FOREIGN PATENT DOCUMENTS

|    |              |         |
|----|--------------|---------|
| EP | 0 788 510 A1 | 7/1997  |
| EP | 0 882 779 A1 | 12/1998 |
| JP | 3 243697     | 10/1991 |
| JP | 5 117680     | 5/1993  |
| JP | 11 013638    | 1/1999  |
| JP | 11 335690    | 12/1999 |
| JP | 2000 17282   | 1/2000  |
| JP | 2001 504547  | 4/2001  |
| JP | 2004 277787  | 10/2004 |

OTHER PUBLICATIONS

European Office Action dated Mar. 10, 2011.

L. Bartha, et al., "Polyfunctional PIB Succinimide Type engine Oil Additives", Lubrication Science, vol. 13, No. 4, Aug. 1, 2001, pp. 313-328, XP009107449.

\* cited by examiner

*Primary Examiner* — Douglas Mc Ginty

(74) *Attorney, Agent, or Firm* — Oblon, Spivak, McClelland, Maier & Neustadt, L.L.P.

(57) **ABSTRACT**

The present invention provides a refrigerator oil composition comprising a base oil which is at least one member selected from mineral oils and synthetic oils, and at least one imide compound, said imide compound in an amount of 0.01 to 5% by mass based on the total amount of the refrigerator oil composition, and also provides a compressor and a refrigeration apparatus using the refrigerator oil composition. The refrigerator oil composition and the compressor and the refrigeration apparatus using the refrigerator oil composition satisfy both sludge dispersibility and prevention of wear and seizing of a sliding part made of aluminum and/or iron.

**21 Claims, No Drawings**

## 1

**REFRIGERATOR OIL COMPOSITION, AND  
REFRIGERATOR COMPRESSOR AND  
REFRIGERATION SYSTEM USING THE  
COMPOSITION**

TECHNICAL FIELD

The present invention relates to a refrigerator oil composition and to a compressor for a refrigerator and a refrigeration apparatus using the refrigerator oil composition. More specifically, the present invention is directed to a refrigerator oil composition containing a base oil and, added thereto, a specific compound, to a compressor for a refrigerator using the refrigerator oil composition and having a sliding part which is made of aluminum and/or iron and which has a coating of an organic coating film or an inorganic coating film as a sliding material, and to a refrigeration apparatus.

BACKGROUND ART

Lubrication of each of sliding parts of a compressor used in a refrigerator is ensured by a refrigerator oil which is compatible with a refrigerant used. When the sliding parts are made of aluminum and/or iron, however, there has still been a problem of wear and seizing. There has also been caused a problem of capillary clogging due to insufficient sludge dispersibility.

To cope with these problems, Patent Document 1 proposes the use of a refrigerator oil composition containing a base oil of a specific polyether and a phosphorothionate such as an alkyl phosphorothionate or an aryl phosphorothionate.

Patent Document 2 proposes a lubricating oil composition for a sliding part, containing a mineral oil and/or a synthetic oil and, added thereto, 0.05 to 5% by weight of a thiol.

With these proposals, however, it has still been impossible to satisfy both sludge dispersibility and performance of wear and seizure prevention of sliding parts.

In this circumstance there is a demand to establish a refrigerator lubricating system which satisfies both sludge dispersibility and prevention of wear and seizing of a sliding part by improving the refrigerator oil or by improving both the refrigerator oil and the lubricating material.

[Patent Document 1] Japanese Unexamined Patent Publication No. 2000-17282

[Patent Document 2] Japanese Unexamined Patent Publication No. H05-117680

DISCLOSURE OF THE INVENTION

The present invention has been made to solve the foregoing problem and has as its object the provision of a refrigerator oil composition which satisfies both sludge dispersibility and prevention of wear and seizing of a sliding part made of aluminum and/or iron, and of a compressor and a refrigeration apparatus using the refrigerator oil composition.

The present inventors have made an earnest study with a view toward accomplishing the above objects and, as a result, have found that the above objects can be fulfilled by using a refrigerator oil composition having a specific composition and, further, by combining the specifically tailored refrigerator oil composition with a specific sliding material coated on at least one of sliding parts in components constituting a compressing mechanism section. The present invention has been completed on the based on such findings.

## 2

Thus, in accordance with the present invention, there are provided:

- (1) A refrigerator oil composition comprising a base oil which is at least one member selected from mineral oils and synthetic oils, and at least one imide compound in an amount of 0.01 to 5% by mass based on the total amount of the refrigerator oil composition;
- (2) A compressor for a refrigerator using a refrigerator oil composition which comprises a base oil which is at least one member selected from mineral oils and synthetic oils, and at least one imide compound in an amount of 0.01 to 5% by mass based on the total amount of the refrigerator oil composition, wherein said compressor has a sliding part made of aluminum and/or iron in components constituting a compression mechanism section, and wherein said sliding part has a coating of a lubricating film forming composition comprising a binder which is a resin containing nitrogen atoms, oxygen atoms and/or sulfur atoms, and at least one member selected from molybdenum disulfide, a fluorine-containing resin, graphite and carbon black; and
- (3) A refrigeration apparatus configured to circulate a refrigerant selected from carbon dioxide, a hydrofluorocarbon, a hydrocarbon and ammonia through a cooling circuit including a compressor, a radiator, an expansion mechanism and an evaporator, said compressor using a refrigerator oil composition comprising a base oil which is selected from mineral oils and synthetic oils and has a kinematic viscosity at 40° C. of 2 to 500 mm<sup>2</sup>/s, and at least one imide compound in an amount of 0.01 to 5% by mass based on the total amount of the refrigerator oil composition, said compressor having a sliding part which is made of an aluminum and/or iron and which has a coating of a lubricating film forming composition comprising a binder which is at least one resin selected from the group consisting of a polyamide, a polyamideimide, a polyimide, a polybenzoazole, a polyphenylene sulfide and a polyacetal, and at least one member selected from molybdenum disulfide, a fluorine-containing resin, graphite and carbon black.

BEST MODE FOR CARRYING OUT THE INVENTION

In the refrigerator oil composition of the present invention, at least one member selected from mineral oils and synthetic oils is used as a base oil. As the mineral oil, there may be mentioned naphthenic mineral oils and paraffinic mineral oils. As the synthetic oil, on the other hand, there may be mentioned, for example, alkylbenzenes, alkylnaphthalenes, poly- $\alpha$ -olefins, polyalkylene glycols, polyoxyalkylene monoethers, polyoxyalkylene diethers, polyvinyl ether-polyalkylene glycol copolymers, polyol esters and polycarbonates.

Among these mineral oils and synthetic oils, polyvinyl ethers, polyalkylene glycols, polyoxyalkylene monoethers, polyoxyalkylene diethers, polyvinyl ether-polyalkylene glycol copolymers, polyol esters and polycarbonates are preferred.

It is preferred that the base oil used in the refrigerator oil composition of the present invention have a kinematic viscosity at 40° C. of 2 to 500 mm<sup>2</sup>/s, more preferably 3 to 300 mm<sup>2</sup>/s. A kinematic viscosity of 2 mm<sup>2</sup>/s or more provides a satisfactory lubrication, while a kinematic viscosity of 500 mm<sup>2</sup>/s or less can reduce a viscosity resistance and, therefore, provides excellent energy saving efficiency and oil returnability.

The imide compound, which is compounded into the refrigerator oil composition of the present invention, is pref-

erably a monoimide compound, a bisimide compound and/or a polyimide compound having 3 or more imide groups in the molecule.

The refrigerator oil composition of the present invention contains at least one of these imide compounds in an amount of 0.01 to 5% by mass, preferably 0.1 to 4% by mass, particularly preferably 0.2 to 2% by mass, based on the total amount of the refrigerator oil composition. When the amount is less than 0.01% by mass, lubricating efficiency and sludge dispersibility are deteriorated. When the amount is greater than 5% by mass, the stability becomes deteriorated.

As the monoimide, there may be preferably mentioned phthalimide, glutarimide, succinimide, nonylphthalimide, nonylglutarimide, laurylglutarimide, nonylsuccinimide, laurylsuccinimide, oleylsuccinimide, stearylsuccinimide, polybutenylsuccinimide, N-((1,2-ethylenediamine)monoethylene)-3-(2-nonyl)succinimide, N-((1,2-ethylenediamine)monoethylene)-3-(2-lauryl)succinimide, N-((1,2-ethylenediamine)monoethylene)-3-(2-octadecenyl)succinimide, N-(piperazinemonoethylene)-3-(2-lauryl)succinimide, N-(piperazinemonoethylene)-3-(2-hexadecenyl)succinimide, boric acid salt of N-((1,2-ethylenediamine)monoethylene)-3-(2-nonyl)succinimide, boric acid salt of N-((1,2-ethylenediamine)monoethylene)-3-(2-lauryl)succinimide and N-((1,2-bis-dihydroxyborooethylenediamino)monoethylene)-3-(2-octadecenyl)succinimide.

As the bisimide, there may be preferably mentioned nonylsuccinic acid bisimide, laurylsuccinic acid bisimide, oleylsuccinic acid bisimide, stearylsuccinic acid bisimide, polybutenylsuccinic acid bisimide, 2,2'bis(3-(2-nonyl)succimino)diethylamine, 2,2'bis(3-(2-lauryl)succinimino)diethylamine and 2,2'bis(3-(2-octadecenyl)succinimino)diethylamine.

A polyimide compound having three or more imide groups in the molecule may also be used.

Among the above imide compounds, nonylphthalimide, laurylglutarimide, oleylsuccinimide, polybutenylsuccinimide, nonylsuccinic acid bisimide, oleylsuccinic acid bisimide, N-((1,2-ethylenediamine)monoethylene)-3-(2-lauryl)succinimide, boric acid salt of N-((1,2-ethylenediamine)monoethylene)-3-(2-lauryl)succinimide, N-(piperazinemonoethylene)-3-(2-lauryl)succinimide and 2,2'bis(3-(2-lauryl)succinimino)diethylamine are particularly preferred for reasons of excellent lubricating efficiency and sludge dispersibility.

The refrigerator oil composition of the present invention may be compounded with a variety of known additives if necessary. It is preferred that the refrigerator oil composition of the present invention contain a phosphorus acid ester as an extreme pressure agent. The term "phosphorus acid ester" as used herein is intended to comprise a phosphate, an acid phosphate, a phosphite, an acid phosphite and amine salts of them.

The phosphate may be, for example, a triaryl phosphate, a trialkyl phosphate, a trialkylaryl phosphate, a triaryalkyl phosphate or a trialkenyl phosphate. Specific examples of the phosphate include triphenyl phosphate, tricresyl phosphate, benzyl diphenyl phosphate, ethyl diphenyl phosphate, tributyl phosphate, ethyl dibutyl phosphate, cresyl diphenyl phosphate, dicesyl phenyl phosphate, ethylphenyl diphenyl phosphate, diethylphenyl phenyl phosphate, propylphenyl diphenyl phosphate, dipropylphenyl phenyl phosphate, triethylphenyl phosphate, tripropylphenyl phosphate, butylphenyl diphenyl phosphate, dibutylphenyl phenyl phosphate, tributylphenyl phosphate, trihexyl phosphate, tri(2-ethyl-

hexyl) phosphate, tridecyl phosphate, trilauryl phosphate, trimyristyl phosphate, tripalmityl phosphate, tristearyl phosphate and trioleyl phosphate.

Specific examples of the acid phosphate include 2-ethylhexyl acid phosphate, ethyl acid phosphate, butyl acid phosphate, oleyl acid phosphate, tetracosyl acid phosphate, isodecyl acid phosphate, lauryl acid phosphate, tridecyl acid phosphate, stearyl acid phosphate and isostearyl acid phosphate.

Specific examples of the phosphite include triethyl phosphate, tributyl phosphite, triphenyl phosphite, tricresyl phosphate, tri(nonylphenyl) phosphite, tri(2-ethylhexyl) phosphate, tridecyl phosphite, trilauryl phosphite, triisoctyl phosphite, diphenylisodecyl phosphite, tristearyl phosphite and trioleyl phosphite.

Specific examples of the acid phosphite include dibutyl hydrogen phosphite, dilauryl hydrogen phosphite, dioleyl hydrogen phosphite, distearyl hydrogen phosphite and diphenyl hydrogen phosphite. Among the above phosphorus acid esters, oleyl acid phosphate and stearyl acid phosphate are particularly preferable.

Amines that form amine salts with the above described phosphates, acid phosphates, phosphites and acid phosphites are exemplified below.

Examples of the monosubstituted amine include butylamine, pentylamine, hexylamine, cyclohexylamine, octylamine, laurylamine, stearylamine, oleylamine and benzylamine. Examples of the disubstituted amine include dibutylamine, dipentylamine, dihexylamine, dicyclohexylamine, dioctylamine, dilaurylamine, distearylamine, dioleylamine, dibenzylamine, stearylmonoethanolamine, decylmonoethanolamine, hexylmonopropanolamine, benzylmonoethanolamine, phenylmonoethanolamine and tolylmonopropanolamine. Examples of the trisubstituted amine include tributylamine, tripentylamine, trihexylamine, tricyclohexylamine, trioctylamine, trilaurylamine, tristearylamine, trioleylamine, tribenzylamine, dioleylmonoethanolamine, dilaurylmonopropanolamine, dioctylmonoethanolamine, dihexylmonopropanolamine, dibutylmonopropanolamine, oleylmonoethanolamine, stearyl-dipropanolamine, lauryldiethanolamine, octyldipropanolamine, butyldiethanolamine, benzylidethanolamine, phenyldiethanolamine, tolylidipropanolamine, xylyldiethanolamine, triethanolamine and tripropanolamine.

It is also preferred that the refrigerator oil composition of the present invention contains an antioxidant and an acid scavenger.

As the antioxidant, there may be mentioned a phenol-based antioxidant and an amine-based antioxidant. To be more specific, it is preferable to use a phenol-based antioxidant such as 2,6-di-tert-butyl-4-methylphenol (DBPC), 2,6-di-tert-butyl-4-ethylphenol, 2,2'-methylenebis(4-methyl-6-tert-butylphenol), 2,4-dimethyl-6-tert-butylphenol and 2,6-di-tert-butylphenol, or an amine-based antioxidant such as N,N'-diisopropyl-p-phenylenediamine, N,N'-di-sec-butyl-p-phenylenediamine, phenyl- $\alpha$ -naphthylamine and N,N'-di-phenyl-p-phenylenediamine. The antioxidant is compounded in the composition in an amount of generally 0.01 to 5% by mass, preferably 0.05 to 3% by mass.

As the acid scavenger, there may be mentioned, for example, phenyl glycidyl ether, an alkyl glycidyl ether, an alkylene glycol glycidyl ether, cyclohexene oxide, an  $\alpha$ -olefin oxide and an epoxy compound such as epoxidized soybean oil. Among these, phenyl glycidyl ether, alkyl glycidyl ether, alkylene glycol glycidyl ether, cyclohexane oxide and  $\alpha$ -olefin oxide are preferred from the standpoint of compatibility.

Each of the alkyl group of the alkyl glycidyl ether and the alkylene group of the alkylene glycol glycidyl ether may be branched and has generally 3 to 30, preferably 4 to 24, particularly 6 to 16 carbon atoms. The  $\alpha$ -olefin oxide used has a total carbon number of generally 4 to 50, preferably 4 to 24, particularly 6 to 16. In the present invention, the above-described acid scavengers may be used singly or in combination of two or more thereof. The compounding amount of the acid scavenger is generally preferably in the range of 0.005 to 5% by mass, particularly preferably 0.05 to 3% by mass, from the standpoint of the acid scavenging effect and the suppression of the sludge generation.

Further, the refrigerator oil composition of the present invention may contain known additives customarily employed in the conventional lubricating oils and may contain, for example, an extreme pressure agent other than those described above. Such "other extreme pressure agent" may be, for example, an organic sulfur compound-based agent such as a monosulfide, a polysulfide, a sulfoxide, a sulfone, a thiosulfinate, a sulfurized fat, a thiocarbonate, a thiophene, a thiazole and a methanesulfonate; a thiophosphate-based agent such as a triester of thiophosphoric acid; a higher fatty acid; a hydroxyarylfatty acid; an ester-based agent such as an ester of a polyhydric alcohol and an acrylate; an organic chlorine compound-based agent such as a chlorinated hydrocarbon and a chlorinated carboxylic acid derivative; an organic fluorine compound-based agent such as a fluorinated aliphatic carboxylic acid, a fluorinated ethylene resin, a fluorinated alkylpolysiloxane and a fluorinated graphite; an alcohol-based agent such as a higher alcohol; a metal compound-based agent such as a naphthenic acid salt (e.g. lead naphthenate), a fatty acid salt (a lead salt of a fatty acid), a thiophosphoric acid salt (zinc dialkyldithiophosphate), a thiocarbamic acid salt, an organomolybdenum compound, an organotin compound, an organogermanium compound and a boric acid ester.

Furthermore, a copper deactivator such as benzotriazole and its derivatives may be compounded into the refrigerator oil composition. The refrigerator oil composition may further comprise other additives such as a load withstanding additive, a chlorine scavenger, a detergent dispersant, a viscosity index improver, an oiliness agent, a rust preventive agent, a corrosion inhibitor, a pour point improver and an antifoaming agent. These additives may be present in the refrigerator oil composition in an amount of 0.1 to 10% by mass, preferably 0.5 to 10% by mass, based on the total amount of the refrigerator oil composition.

The compressor for a refrigerator according to the present invention has at least one sliding part made of aluminum and/or iron in components constituting a compression mechanism section thereof. The compressor is characterized in that the at least one sliding part has a coating of a lubricating material. As the lubricating material, an organic coating film or an inorganic coating film is suitably used.

The organic coating film is more preferably composed of a lubricating film forming composition containing as a binder a resin having a heat distortion temperature of 100°C. or more and a solid lubricating agent.

The term "heat distortion temperature (HDT)" as used herein is intended to refer to a temperature at which the plastic is deformed when it is heated at a constant rate with a given load being applied thereto and is a temperature as determined in accordance with Heat Distortion Temperature Test specified in ASTM D648 (1.8 MPa).

The inorganic coating film may be an inorganic material film and/or a metal plating film. The inorganic material may be graphite, diamond-like carbon (DLC), titanium carbide

(TiC), boron nitride (BN), etc. The metal plating film may be preferably at least one member selected from nickel platings, molybdenum platings, tin platings, chromium platings, KANIFLON platings, KANIZEN platings, iron-based alloy platings, aluminum-based alloy platings and copper-based alloy platings.

These inorganic material films and metal plating films may be preferably formed by a vacuum deposition method. Examples of the vacuum deposition method include a chemical vapor deposition (CVD) method (e.g. a plasma CVD method) and a physical vapor deposition (PVD) method (e.g. an ion plating method and a sputtering method). As a method for forming a metal plating film, there may be used electrolytic plating and electroless plating.

When the above-described lubricating film forming composition is used as the lubricating material in the present invention, the sliding part made of aluminum and/or iron exhibits significantly improved lubricity at the start of and during the operation of the compressor for a refrigerator because of an interaction between the lubricating material and the imide compound. Therefore, the use of the lubricating film forming composition is particularly preferred.

The binder used in the lubricating film forming composition is preferably a resin having a heat distortion temperature of 100°C. or more, more preferably 150°C. or more, still more preferably 200°C. or more, particularly preferably 250°C. or more.

More specifically, the binder is preferably a resin containing nitrogen atoms, oxygen atoms and/or sulfur atoms. Examples of the resin include an epoxy resin, a phenol resin, a fluorine-containing resin, an unsaturated polyester, a polyacetal, a polyimide, a polyamideimide, a polyamide, a polycarbonate, a polysulfone, a polyphenylene sulfide and a polybenzoazole. Above all, a polyamide, a polyimide, a polyamideimide, a polybenzoazole, a polyphenylene sulfide and a polyacetal are particularly preferred for reasons of excellent heat stability.

As the polyamide, there may be mentioned, for example, an aromatic polyamide, a polyether amide and a modified product thereof. As the polyimide, there may be mentioned, for example, an aromatic polyimide, a polyether imide and a modified product thereof. As the polyamideimide, there may be mentioned, for example, an aromatic polyamideimide and a modified product thereof. As the polybenzoazole, there may be suitably mentioned, for example, a polybenzimidazole. These resins may be used by themselves or as a mixture of two or more thereof.

In the present invention, the above-described binder is contained in the lubricating film forming composition. The composition is applied to at least one sliding part made of aluminum and/or iron in components constituting a compression mechanism section. The binder is preferably present in the lubricating film forming composition in an amount of 20 to 100% by mass based on the total amount of the lubricating film forming composition. When the amount is 20% by mass or more, a solid lubricating agent which is mentioned later can be firmly supported within the lubricating film, so that sufficient lubricity can be obtained. The amount of the binder in the lubricating film forming composition is more preferably in a range of 20 to 80% by mass in compounding the solid lubricating agent.

Any solid lubricating agent may be used as long as it can exhibit lubricating action in a solid state. Specific examples of the solid lubricating agent include graphite, carbon black, molybdenum disulfide, tungsten sulfide, fluorine-containing polymers (particularly fluorine-containing resins), boron nitride and graphite. Among these, molybdenum disulfide,

fluorine-containing resins, graphite and carbon black are preferred. These solid lubricating agents may be used by themselves or as a mixture of two or more thereof.

The average particle diameter of the solid lubricating agent contained in the lubricating film is not specifically limited. For reasons of formation of dense lubricating films, it is preferred that the average particle diameter be in a range of 1 to 100  $\mu\text{m}$ .

The content of the solid lubricating agent is preferably in a range of 20 to 80 parts by mass per 100 parts by mass of the binder resin. When the content is 20 parts by mass or more, sufficient lubricity can be obtained. When the content is not greater than 80 parts by mass, no reduction of the action of binding the solid lubricating agent in the lubricating film due to a decrease of the content of the binder occurs and, therefore, no abrasion or exfoliation of the solid lubricating agent occurs. The content of the solid lubricating agent is more preferably in a range of 30 to 70 parts by mass per 100 parts by mass of the binder resin.

It is preferred that the lubricating film forming composition contain a film forming aid. Illustrative of suitable film forming aids are, for example, epoxy group-bearing compounds and silane coupling agents. The film forming aid serves to improve the action of holding the solid lubricating agent.

The film forming aid is preferably used in such an amount that the ratio by mass of the binder resin to the film forming aid is in a range of 99:1 to 70:30.

A variety of known additives may be compounded into the lubricating film forming composition if necessary. For example, an extreme pressure agent such as a phosphate (e.g. tricresyl phosphate (TCP)) and a phosphite (e.g. tri(nonylphenyl)phosphite); an antioxidant such as a phenol-based and amine-based antioxidant; a stabilizer such as phenyl glycidyl ether, cyclohexene oxide, epoxidized soy bean oil; and a copper deactivator such as benzotriazole and its derivatives, may be compounded into the lubricating film forming composition as desired. In addition, the lubricating film forming composition may comprise a load withstanding additive, a chlorine scavenger, a detergent dispersant, a viscosity index improver, an oiliness agent, a rust preventive agent, a corrosion inhibitor, a pour point improver, etc. These additives may be present in the refrigerator oil composition in an amount of 0.1 to 10% by mass, preferably 0.5 to 10% by mass, based on the total amount of the refrigerator oil composition.

The thickness of the lubricating film is not specifically limited as long as the effect of the present invention may be ensured, but is preferably in a range of 2 to 50  $\mu\text{m}$ . When the thickness is 2  $\mu\text{m}$  or more, sufficient lubricity can be ensured. When the thickness is 50  $\mu\text{m}$  or less, fatigue resistance can be maintained. From these points of view, the thickness of the lubricating film is more preferably in a range of 4 to 25  $\mu\text{m}$ .

The lubricating film forming composition is applied to at least one sliding part made of aluminum and/or iron in components constituting a compression mechanism section. The coating method is not specifically limited. Examples of the coating method include a method in which a lubricating film forming composition is prepared by dispersing a solid lubricating agent in a solution of the above-described binder in an organic solvent and in which the obtained composition is directly applied to a sliding part made of aluminum and/or iron; and a method in which a sliding part made of aluminum

and/or iron is immersed in the above-obtained composition. The sliding part made of aluminum and/or iron on which the composition has been applied is then treated by drying or the like method to remove the solvent, thereby forming a lubricating film.

The refrigerator oil of the present invention may be used for a variety of refrigerants. Suitable examples of the refrigerant include a carbon dioxide refrigerant, a hydrocarbon-based refrigerant, an ammonia-based refrigerant and a hydrofluorocarbon-based refrigerant. Among these refrigerants, a carbon dioxide refrigerant is particularly suitably used.

It is preferred that the compressor for a refrigerator according to the present invention be a compressor which uses the above-described refrigerator oil composition and which has a sliding part made of aluminum and/or iron in components constituting a compression mechanism section, with the sliding part having a coating of a lubricating film forming composition containing a binder, which is a resin containing nitrogen atoms, oxygen atoms and/or sulfur atoms, and at least one member selected from molybdenum disulfide, a fluorine-containing resin, graphite and carbon black. The compression mechanism of the compressor preferably uses at least one operation type selected from a scroll type, a rotary type, a swing type and a piston type. In addition, the term "components constituting a compression mechanism section" as used herein is intended to comprise, for example, a piston and a cylinder in the case of a reciprocating piston compressor. The above-described lubricating film forming composition is coated on such a sliding part or parts made of aluminum and/or iron so that lubricity of the sliding part or parts made of aluminum and/or iron is ensured by using the refrigerator oil composition.

The present invention also provides a refrigeration apparatus configured to circulate a refrigerant selected from carbon dioxide, a hydrofluorocarbon, a hydrocarbon and ammonia through a cooling circuit including the above-described compressor, a radiator, an expansion mechanism and an evaporator.

It is preferred that the moisture content in a system of the refrigeration apparatus be not greater than 300 ppm for reasons of suppressing hydrolysis and corrosion. It is also preferred that the residual air content be not greater than 50 ppm for suppressing oxidative deterioration.

## EXAMPLES

The present invention will be next described in more detail by way of examples but is not restricted to these examples in any way.

Refrigerator oil compositions were evaluated by the following methods.

### (1) Closed Block on Ring Abrasion Test

Block abrasion width (mm) was determined under the following conditions. Load: 100 N; Rotating speed: 1,000 rpm; Time: 20 minutes; Temperature: 50°C.; Refrigerant: carbon dioxide; Refrigerant pressure: 1 MPa; Block/ring: A4032/MoNiChro cast iron.

### (2) Dispersibility Test

A sample oil was mixed with 0.5% of barium sulfonate-based rust preventive agent and maintained at -5°C. Whether or not precipitation occurred was checked.

Examples 1 to 15 and Comparative Examples 1 to 3

Eighteen refrigerator oil compositions having formulations shown in Table 1 were prepared and evaluated by the above methods. The results are summarized in Table 1.

TABLE 1

| Compounding amount<br>(% by mass) | Example<br>1                                              | Example<br>2          | Example<br>3          | Example<br>4                | Example<br>5                | Example<br>6                |
|-----------------------------------|-----------------------------------------------------------|-----------------------|-----------------------|-----------------------------|-----------------------------|-----------------------------|
| Sample Oil No.                    | Sample<br>Oil 1                                           | Sample<br>Oil 2       | Sample<br>Oil 3       | Sample<br>Oil 4             | Sample<br>Oil 5             | Sample<br>Oil 6             |
| Base Oil                          | A1<br>A2<br>A3<br>A4<br>A5<br>A6                          | 96.5                  | 96.5                  | 96.5                        | 96.5                        | 96.5                        |
| Imide<br>Compound                 | B1<br>B2<br>B3<br>B4<br>B5<br>B6<br>B7<br>B8<br>B9<br>B10 | 1                     | 1                     | 1                           | 1                           | 1                           |
| Extreme<br>Pressure Agent         | C1                                                        | 1                     | 1                     | 1                           | 1                           | 1                           |
| Acid Scavenger                    | C2                                                        | 1                     | 1                     | 1                           | 1                           | 1                           |
| Antioxidant                       | C3                                                        | 0.5                   | 0.5                   | 0.5                         | 0.5                         | 0.5                         |
| Antifoaming<br>Agent              | C4                                                        | 0.001                 | 0.001                 | 0.001                       | 0.001                       | 0.001                       |
| Block Abrasion Width<br>(mm)      |                                                           | 1.2                   | 0.9                   | 1.4                         | 1.2                         | 1.1                         |
| Dispersibility Test               |                                                           | No precipi-<br>tation | No precipi-<br>tation | No precipi-<br>tation       | No precipi-<br>tation       | No precipi-<br>tation       |
| Compounding amount<br>(% by mass) | Example<br>7                                              | Example<br>8          | Example<br>9          | Example<br>10               | Example<br>11               | Example<br>12               |
| Sample Oil No.                    | Sample<br>Oil 7                                           | Sample<br>Oil 8       | Sample<br>Oil 9       | Sample<br>Oil 10            | Sample<br>Oil 11            | Sample<br>Oil 12            |
| Base Oil                          | A1<br>A2<br>A3<br>A4<br>A5<br>A6                          | 96.5                  | 96.5                  | 96.5                        | 96.5                        | 96.5                        |
| Imide<br>Compound                 | B1<br>B2<br>B3<br>B4<br>B5<br>B6<br>B7<br>B8<br>B9<br>B10 | 1                     | 1                     | 1                           | 1                           | 1                           |
| Extreme<br>Pressure Agent         | C1                                                        | 1                     | 1                     | 1                           | 1                           | 1                           |
| Acid Scavenger                    | C2                                                        | 1                     | 1                     | 1                           | 1                           | 1                           |
| Antioxidant                       | C3                                                        | 0.5                   | 0.5                   | 0.5                         | 0.5                         | 0.5                         |
| Antifoaming<br>Agent              | C4                                                        | 0.001                 | 0.001                 | 0.001                       | 0.001                       | 0.001                       |
| Block Abrasion Width<br>(mm)      |                                                           | 1.5                   | 1.3                   | 1.3                         | 1.2                         | 1.2                         |
| Dispersibility Test               |                                                           | No precipi-<br>tation | No precipi-<br>tation | No precipi-<br>tation       | No precipi-<br>tation       | No precipi-<br>tation       |
| Compounding amount<br>(% by mass) | Example<br>13                                             | Example<br>14         | Example<br>15         | Comparative<br>Example<br>1 | Comparative<br>Example<br>2 | Comparative<br>Example<br>3 |
| Sample Oil No.                    | Sample<br>Oil 13                                          | Sample<br>Oil 14      | Sample<br>Oil 15      | Sample<br>Oil 16            | Sample<br>Oil 17            | Sample<br>Oil 18            |
| Base Oil                          | A1<br>A2<br>A3<br>A4<br>A5<br>A6                          | 96.5                  | 96.5                  | 97.5                        | 97.5                        | 97.5                        |
| Imide<br>Compound                 | B1<br>B2<br>B3<br>B4                                      |                       |                       |                             |                             |                             |

TABLE 1-continued

|                           |    |                  |                  |                  |                        |                        |
|---------------------------|----|------------------|------------------|------------------|------------------------|------------------------|
| B5                        |    |                  |                  |                  |                        |                        |
| B6                        |    |                  |                  |                  |                        |                        |
| B7                        |    |                  |                  |                  |                        |                        |
| B8                        | 1  | 1                | 1                |                  |                        |                        |
| B9                        |    |                  |                  |                  |                        |                        |
| B10                       |    |                  |                  |                  |                        |                        |
| Extreme Pressure Agent    | C1 | 1                | 1                | 1                | 1                      | 1                      |
| Acid Scavenger            | C2 | 1                | 1                | 1                | 1                      | 1                      |
| Antioxidant               | C3 | 0.5              | 0.5              | 0.5              | 0.5                    | 0.5                    |
| Antifoaming Agent         | C4 | 0.001            | 0.001            | 0.001            | 0.001                  | 0.001                  |
| Block Abrasion Width (mm) |    | 1.2              | 1.7              | 1.9              | 5.2                    | 3.8                    |
| Dispersibility Test       |    | No precipitation | No precipitation | No precipitation | Precipitation Occurred | Precipitation Occurred |
|                           |    |                  |                  |                  | Precipitation Occurred | Precipitation Occurred |

## Remarks:

A1: Polyvinyl ether (kinematic viscosity at 40° C.: 68.1 mm<sup>2</sup>/s)A2: Polyalkylene glycol (kinematic viscosity at 40° C.: 46.7 mm<sup>2</sup>/s)A3: Polyvinyl ether-polyalkylene glycol copolymer (molar ratio: 1/1): (kinematic viscosity at 40° C.: 75.2 mm<sup>2</sup>/s)A4: Polyol ester (kinematic viscosity at 40° C.: 68.5 mm<sup>2</sup>/s)A5: Polycarbonate (kinematic viscosity at 40° C.: 67.9 mm<sup>2</sup>/s)A6: Paraffinic mineral oil (kinematic viscosity at 40° C.: 101.0 mm<sup>2</sup>/s)

B1: Nonylphthalimide

B2: Laurylglutarimide

B3: Oleylsuccinimide

B4: Polybutenylsuccinimide

B5: Nonylsuccinic acid bisimide

B6: Oleylsuccinic acid bisimide

B7: N-(1,2-ethylenediamine)monoethylene)-3-(2-lauryl)succinimide

B8: Boric acid salt of N-((1,2-ethylenediamine)monoethylene)-3-(2-lauryl)succinimide

B9: N-(piperazinemonoethylene)-3-(2-lauryl)succinimide

B10: 2,2'-Bis(3-(2-lauryl)succinimino)diethylamine

C1: Tricresyl phosphate (TCP)

C2: C<sub>14</sub>- $\alpha$ -Olefin oxide

C3: 2,6-Di-tert-butyl-4-methylphenol (DBPC)

C4: Silicon-based antifoaming agent

As is evident from Table 1, the refrigerator oil composition of the present invention is excellent in both sludge dispersibility and prevention of wear and seizing of sliding parts, made of aluminum and/or iron, of a compressor for a refrigerator.

A lubricating film forming composition containing a polyamideimide as a binder and a mixture of molybdenum disulfide and polytetrafluoroethylene (PTFE) as a solid lubricating agent (ratio of polyamideimide/molybdenum disulfide/PTFE=100/25/25 (parts by mass)) was applied to sliding parts, made of aluminum and/or iron, in components constituting a compression mechanism section to a thickness of 30  $\mu$ m. The coated films were each processed to a thickness of 10 to 20  $\mu$ m and surface roughness Rz (10-point average roughness) of 3.2  $\mu$ m or less. Using each of the fifteen refrigerator oil compositions obtained in Examples 1 to 15, the compressor for a refrigerator having such sliding parts was operated. At the start of and during the operation of the compressor, lubricity of the aluminum sliding part and the iron sliding part was evaluated. It was found that the fifteen refrigerator oil compositions of Examples 1 to 15 showed excellent lubricity in both the aluminum and iron sliding parts.

## INDUSTRIAL APPLICABILITY

The refrigerator oil composition according to the present invention, and a compressor and a refrigeration apparatus using the refrigerator oil composition may be used in a refrigerator of an open type, a semi-close type or a close type and are suitably used in a refrigeration system (such as a car air conditioner, a gas heat pump, an air conditioner, a refrigerator, a vending machine and a showcase), a water heater system and a floor heating system.

35

The invention claimed is:

1. A refrigerator oil composition, consisting of:
  - (a) a base oil which is at least one member selected from the group consisting of naphthenic mineral oils, paraffinic mineral oils, alkylbenzenes, alkylnaphthalenes, poly- $\alpha$ -olefins, polyalkylene glycols, polyoxyalkylene monoethers, polyoxyalkylene diethers, polyvinyl ethers, polyvinyl ether-polyalkylene glycol copolymers, polyol esters and polycarbonates,
  - (b) at least one imide compound in an amount of 0.01 to 5% by mass based on the total amount of the refrigerator oil composition, and
  - (c) optionally, one or more additives selected from the group consisting of a phosphorus acid ester, an antioxidant, an acid scavenger, an organic sulfur-compound based agent, a thiophosphate-based agent, a higher fatty acid, a hydroxyarylfatty acid, an ester-based agent, an organic chlorine compound-based agent, a fluorinated aliphatic carboxylic acid, a fluorinated ethylene resin, a fluorinated alkylpolysiloxane, a fluorinated graphite, an alcohol-based agent, a metal compound-based agent, a copper deactivator, a load withstanding additive, a chlorine scavenger, a detergent dispersant, a viscosity index improver, an oiliness agent, a rust preventive agent, a corrosion inhibitor, a pour point improver and an anti-foaming agent.

2. The refrigerator oil composition as defined in claim 1, wherein said base oil has a kinematic viscosity at 40° C. of 2 to 500 mm<sup>2</sup>/s.

3. The refrigerator oil composition as defined in claim 1, wherein said imide compound is at least one member selected

40

45

50

55

## 13

from the group consisting of monoimide compounds, bisimide compounds and polyimide compounds having 3 or more imide groups in the molecule.

4. The refrigerator oil composition as defined in claim 1, which contains the phosphorus acid ester.

5. The refrigerator oil composition as defined in claim 1, which contains at least one member selected from the antioxidant and the acid scavenger.

6. The refrigerator oil composition as defined in claim 1, which contains 0.1 to 4% by mass of the imide compound.

7. The refrigerator oil composition as defined in claim 1, which contains 0.2 to 2% by mass of the imide compound.

8. The refrigerator oil composition as defined in claim 1, wherein the imide compound is at least one compound selected from the group consisting of phthalimide, glutarimide, succinimide, nonylphthalimide, nonylglutarimide, laurylglutarimide, nonylsuccinimide, laurylsuccinimide, oleylsuccinimide, stearylsuccinimide, polybutenylsuccinimide, N-((1,2-ethylenediamine)monoethylene)-3-(2-nonyl)succinimide, N-((1,2-ethylenediamine)monoethylene)-3-(2-lauryl)succinimide, N-((1,2-ethylenediamine)monoethylene)-3-(2-octadecenyl)succinimide, N-(piperazinemonoethylene)-3-(2-lauryl)succinimide, N-(piperazinemonoethylene)-3-(2-hexadecenyl)succinimide, boric acid salt of N-((1,2-ethylenediamine)monoethylene)-3-(2-nonyl)succinimide, boric acid salt of N-((1,2-ethylenediamine)monoethylene)-3-(2-lauryl)succinimide and N-((1,2-bis-dihydroxybороethylenediamino)monoethylene)-3-(2-octadecenyl)succinimide.

9. The refrigerator oil composition as defined in claim 1, wherein the imide compound is at least one compound selected from the group consisting of nonylsuccinic acid bisimide, laurylsuccinic acid bisimide, oleylsuccinic acid bisimide, stearylsuccinic acid bisimide, polybutenylsuccinic acid bisimide, 2,2'bis(3-(2-nonyl)-succimino)diethylamine, 2,2'bis(3-(2-lauryl)succimino)diethylamine and 2,2'bis(3-(2-octadecenyl)succimino)diethylamine.

10. The refrigerator oil composition as defined in claim 1, wherein the imide compound is at least one compound selected from the group consisting of nonylphthalimide, laurylglutarimide, oleylsuccinimide, polybutenylsuccinimide, nonylsuccinic acid bisimide, oleylsuccinic acid bisimide, N-((1,2-ethylenediamine)monoethylene)-3-(2-lauryl)succinimide, boric acid salt of N-((1,2-ethylenediamine)monoethylene)-3-(2-lauryl)succinimide, N-(piperazinemonoethylene)-3-(2-lauryl)succinimide and 2,2'bis(3-(2-lauryl)succimino)diethylamine.

11. The refrigerator oil composition as defined in claim 1, wherein the base oil contains at least one member selected

## 14

from the group consisting of polyvinyl ethers, polyalkylene glycols, polyoxyalkylene monoethers, polyoxyalkylene diethers, polyvinyl ether-polyalkylene glycol copolymers, polyol esters and polycarbonates.

5 12. The refrigerator oil composition as defined in claim 1, wherein the base oil contains at least one naphthenic mineral oil.

10 13. The refrigerator oil composition as defined in claim 1, wherein the base oil contains at least one paraffinic mineral oil.

14. The refrigerator oil composition as defined in claim 1, wherein the base oil contains at least one member selected from the group consisting of alkylbenzenes, alkynaphthalenes and poly- $\alpha$ -olefins.

15 15. The refrigerator oil composition as defined in claim 1, wherein the base oil contains at least one member selected from the group consisting of polyalkylene glycols, polyoxyalkylene monoethers, polyoxyalkylene diethers, polyvinyl ethers, polyvinyl ether-polyalkylene glycol copolymers, 20 polyol esters and polycarbonates.

16. The refrigerator oil composition as defined in claim 1, which consists of said base oil (a) and said at least one imide compound (b).

25 17. The refrigerator oil composition as defined in claim 1, which contains (c).

18. A compressor for a refrigerator which comprises the refrigerator oil composition as defined in claim 1, wherein said compressor has a sliding part made of aluminum and/or iron in components constituting a compression mechanism 30 section, and wherein said sliding part has a coating of a lubricating film forming composition comprising a binder which is a resin containing nitrogen atoms, oxygen atoms and/or sulfur atoms, and at least one member selected from molybdenum disulfide, a fluorine-containing resin, graphite and carbon black.

19. The compressor for a refrigerator as defined in claim 18, wherein said compressor compresses a refrigerant selected from carbon dioxide, a hydrofluorocarbon, a hydrocarbon and ammonia.

40 20. The compressor for a refrigerator as defined in claim 18, wherein the compression mechanism of said compressor uses at least one operation type selected from a scroll type, a rotary type, a swing type and a piston type.

21. A refrigeration apparatus configured to circulate a 45 refrigerant selected from carbon dioxide, a hydrofluorocarbon, a hydrocarbon and ammonia through a cooling circuit including the compressor of claim 18, a radiator, an expansion mechanism and an evaporator.

\* \* \* \* \*